

1

2,753,240

**PROCESS OF REACTING AMINOALKYLATED CELLULOSIC TEXTILES WITH 8-HYDROXY-QUINOLINE SULFONIC ACIDS AND METALS FORMING CHELATE RINGS AND PRODUCTS THEREOF**

Wilson A. Reeves and John D. Guthrie, New Orleans, La., assignors to the United States of America as represented by the Secretary of Agriculture

No Drawing. Application April 10, 1953,  
Serial No. 348,136

12 Claims. (Cl. 8—129)

(Granted under Title 35, U. S. Code (1952), sec. 266)

A non-exclusive, irrevocable, royalty-free license in the invention herein described, for all governmental purposes, throughout the world, with the power to grant sublicenses for such purposes, is hereby granted to the Government of the United States of America.

This invention relates to modified aminoalkylated cellulosic textiles such as slivers, yarns, threads and fabrics. More particularly, the invention provides aminoalkylated cellulosic textiles containing aryl chelate groups and such textiles to which rot resistance, ultraviolet fluorescence, and the like properties are imparted by metal atoms bound into chelate rings attached to the molecules of the textiles.

As herein employed, the term "aminoalkylated cellulosic textile" refers to a cellulosic textile in which alcoholic hydrogen atoms have been replaced by aminoalkyl radicals. Such textiles are characterized by a marked affinity for acid dyestuffs and other valuable properties. Various processes of preparing aminoalkylated cellulosic textiles are known. U. S. 2,459,222 describes a particularly suitable process of preparing such textiles by reacting a cellulosic textile with 2-aminoethyl sulfuric acid in the presence of aqueous alkali. Aminopropylated textiles produced by reacting cellulosic textiles with 3-aminopropyl sulfuric acid by a similar procedure have similar chemical properties.

The aminoalkylated cellulosic textiles can suitably be employed in the present process in the form of slivers, yarns, threads, or fabric.

In general, the process of the present invention comprises reacting an aminoalkylated cellulosic textile with an aryl sulfonic acid containing chelate groups (i. e., "Atomic groups capable of forming rings by one or two coordinate bonds," Hackh's Chemical Dictionary) dissolved in a dilute aqueous weak acid, until sulfonic acid salts of the amino groups of the textile are formed.

The reaction produces novel chelate group-containing textiles which have physical properties comparable to the aminoalkylated cellulosic textiles from which they are produced. The chelate group-containing textiles also have the capacity of selectively removing polyvalent metals from aqueous solutions of salts of the metals and have numerous uses in addition to those known for aminoalkylated textiles.

Fluorescent textiles are produced in accordance with this invention, in general, by reacting the chelate group-containing textiles with metals that fluoresce when chelated. The reaction is preferably conducted by contacting the textile with an aqueous solution having a pH of from about 3 to 7 containing a soluble salt of the metal. Textiles which are both rot resistant and fluorescent are produced by contacting the chelate group-containing textiles with aqueous solutions of copper salts.

Fluorescent and/or rot resistant textiles produced in

2

accordance with this invention exhibit a marked affinity for acid dyes.

The dilute aqueous weak acid solutions of an aryl sulfonic acid containing a chelate group preferably contain enough of a water soluble acid, preferably a water soluble saturated fatty acid, such as formic, acetic or propionic acid, to make the water solution acetic and from about 0.5% to 5% of a water soluble aryl sulfonic acid containing one or more chelate groups.

Suitable aryl sulfonic acids comprise sulfonic acids which are soluble in water to the extent of at least 0.5% and which contain chelate groups capable of forming 5 or 6 membered rings by the attachment of a metal atom to members of groups such as imino, oxime, hydroxyl, or mercaptyl groups. Preferred sulfonic acids include 8-hydroxyquinoline-5-sulfonic acid, 8-hydroxyquinoline-4-sulfonic acid, and the like. 8-hydroxyquinoline-5-sulfonic acid is particularly suitable.

The reaction between the aminoalkylated cellulosic textile and the aryl sulfonic acid can suitably be conducted at temperatures of from about 25 to 100° C. The reaction is preferably conducted at from 60 to 80° C.

The reaction between the chelate group-containing textiles and a metal salt can suitably be conducted at temperatures of from about 25 to 100° C. The reaction is preferably conducted at from about 40 to 80° C.

Suitable metal salts include zinc acetate, zinc sulfate, copper acetate, copper sulfate, bismuth subnitrate, ferric chloride, and the like. The zinc and copper acetates are preferred.

Aqueous solutions of the metal salts preferably have a pH of from about 4 to 6.

The following examples are illustrative of the invention:

35

*Example 1*

An aminoalkylated cellulosic textile was reacted with 8-hydroxyquinoline-5-sulfonic acid. The textile was immersed for about 15 minutes in a water solution containing 1% of the sulfonic acid and 0.5% of acetic acid and maintained at about 70° C. The so reacted textile was washed free of reactants with water. The aminoalkylated textile used was a 48 by 48 cotton sheeting which had been aminoethylated to a nitrogen content of 0.8% by the process of Patent No. 2,459,222.

The chelate group-containing fabric produced by the reaction constituted a cellulosic textile in which alcoholic hydrogen atoms have been replaced by 8-hydroxyquinoline-5-SO<sub>3</sub>H.H<sub>2</sub>NCH<sub>2</sub>CH<sub>2</sub>-radicals. This fabric exhibited physical properties and an affinity for acid dyes comparable to the aminoalkylated fabric from which it was produced.

A portion of this chelate group-containing fabric was immersed for 2 minutes in a water solution containing 0.5% acetic acid and 5% copper acetate maintained at a temperature of 70-75° C., removed, and washed free of the solution with water.

The copper-containing fabric so produced constituted a cellulosic textile in which alcoholic hydrogen atoms have been replaced by 8-hydroxyquinoline-5-SO<sub>3</sub>H.H<sub>2</sub>NCH<sub>2</sub>CH<sub>2</sub>-radicals in which the quinoline portion contains an atom of copper bound into a chelate ring. This fabric exhibited physical properties and an affinity for acid dyes comparable to the aminoalkylated fabric from which it was produced. In ordinary light the fabric had a light green color, and in ultraviolet light the fabric fluoresced to a deep wine red color.

A comparison of the rot resistance or mildew resistance of the fabric (determined by the soil burial test "A. S. T. M. Standards," Philadelphia, 1951, pp. 140-1 and pp. 142 (D39-49); pp. 157-60 (D1175-51T)) with untreated 48 x 48 cotton sheeting and aminoalkylated

48 x 48 cotton sheeting is reported in the following table:

| Fabric            | Breaking strength (lb.) |      |      |      |      |      |
|-------------------|-------------------------|------|------|------|------|------|
|                   | Days in soil bed        |      |      |      |      |      |
|                   | 0                       | 7    | 14   | 24   | 33   | 41   |
| Untreated         | 72.8                    | 3.9  |      |      |      |      |
| Aminated          | 60.0                    | 30.0 | 5.7  |      |      |      |
| Aminated-Chelated | 51.4                    | 42.1 | 26.1 | 16.8 | 17.5 | 15.0 |

*Example 2*

A zinc-containing fabric was prepared from a portion of the same chelate group-containing fabric by the process of Example 1 using an equivalent amount of zinc acetate in place of the copper acetate.

The zinc-containing fabric so produced constituted a cellulosic textile in which alcoholic hydrogen atoms have been replaced by 8-hydroxyquinoline-5-SO<sub>3</sub>H.H<sub>2</sub>NCH<sub>2</sub>CH<sub>2</sub>-radicals in which the quinoline portion contains an atom of zinc bound into a chelate ring. This fabric exhibited physical properties and an affinity for acid dyes comparable to the aminoalkylated cellulosic textile from which it was produced. In ordinary light, the fabric had a light yellow color, and in ultraviolet light the fabric fluoresced to a bright yellow color.

*Example 3*

A bismuth-containing fiber was prepared from a portion of the same chelate group-containing fabric by the process of Example 1 using approximately an equivalent amount of bismuth subnitrate (BiONO<sub>3</sub>.H<sub>2</sub>O) in place of the copper acetate.

The bismuth-containing fabric so produced constituted a cellulosic textile in which alcoholic hydrogen atoms have been replaced by 8-hydroxyquinoline-5-SO<sub>3</sub>H.H<sub>2</sub>NCH<sub>2</sub>CH<sub>2</sub>-radicals in which the quinoline portion contains an atom of bismuth bound into a chelate ring. This fabric exhibited physical properties and an affinity for acid dyes comparable to the aminoalkylated cellulosic textile from which it was produced. In ordinary light, the fabric had a yellow color, and in ultraviolet light the fabric was red.

We claim:

1. A cellulosic textile in which alcoholic hydrogen atoms of the cellulose molecules have been replaced by 8-hydroxyquinoline-5-SO<sub>3</sub>H.H<sub>2</sub>NCH<sub>2</sub>CH<sub>2</sub>-radicals.
2. A cellulosic textile in which alcoholic hydrogen atoms of the cellulose molecules have been replaced by 8-hydroxyquinoline-5-SO<sub>3</sub>H.H<sub>2</sub>NCH<sub>2</sub>CH<sub>2</sub>-radicals in which the quinoline portion contains an atom of copper bound into a chelate ring.
3. A cellulosic textile in which alcoholic hydrogen atoms of the cellulose molecules have been replaced by 8-hydroxyquinoline-5-SO<sub>3</sub>H.H<sub>2</sub>NCH<sub>2</sub>CH<sub>2</sub>-radicals in

which the quinoline portion contains an atom of zinc bound into a chelate ring.

4. A cellulosic textile in which alcoholic hydrogen atoms of the cellulose molecules have been replaced by 8-hydroxyquinoline-5-SO<sub>3</sub>H.H<sub>2</sub>NCH<sub>2</sub>CH<sub>2</sub>-radicals in which the quinoline portion contains an atom of bismuth bound into a chelate ring.

5. A cellulosic textile in which alcoholic hydrogen atoms of the cellulose molecules have been replaced by 8-hydroxyquinoline-5-SO<sub>3</sub>H.H<sub>2</sub>NCH<sub>2</sub>CH<sub>2</sub>-radicals in which the quinoline portion contains an atom of polyvalent metal bound into a chelate ring, said polyvalent metal being one which fluoresces when so bound in a chelate ring.

15 6. A process comprising, reacting an amino-lower-alkylated cellulosic textile with a dilute aqueous weak acid solution of a compound from the group consisting of 8-hydroxyquinoline-5-sulfonic acid and 8-hydroxy-quinoline-4-sulfonic acid until amino groups of the cellulosic textile are converted to sulfonic acid salts.

10 7. A process comprising reacting an amino-lower-alkylated cellulosic textile with a dilute aqueous weak acid solution of a compound from the group consisting of 8-hydroxyquinoline-5-sulfonic acid and 8-hydroxy-quinoline-4-sulfonic acid until amino groups of the cellulosic textile are converted to sulfonic acid salts, and reacting the textile so produced with a dilute aqueous weak acid solution of a salt of polyvalent metal capable of forming fluorescent chelate ring-containing compounds to produce a textile having polyvalent metal atoms bound in chelate rings attached to the molecules of said textile.

15 8. A cellulosic textile in which alcoholic hydrogen atoms of the cellulose molecules have been replaced by 8-hydroxyquinoline-5-SO<sub>3</sub>H.H<sub>2</sub>NCH<sub>2</sub>CH<sub>2</sub>-radicals, in which the quinoline portion contains an atom of a polyvalent metal from the group consisting of copper, zinc, bismuth, and iron bound into a chelate ring.

20 9. A process comprising reacting an amino-lower-alkylated cellulosic textile with a dilute aqueous weak acid solution of 8-hydroxyquinoline-5-sulfonic acid until amino groups of the cellulosic textile are converted to sulfonic acid salts, and then reacting the textile so produced with a dilute weak acid solution of a salt of a polyvalent metal from the group consisting of copper, zinc, bismuth, and iron to produce a textile having metal atoms bound in chelate rings attached to the molecules of said textile.

25 10. The process of claim 9 in which the metal salt is copper acetate.

11. The process of claim 9 in which the metal salt is zinc acetate.

12. The process of claim 9 in which the metal salt is bismuth subnitrate.

55 References Cited in the file of this patent

UNITED STATES PATENTS  
2,459,222 Guthrie Jan. 18, 1949